

## UNITED STATES PATENT OFFICE

2,170,253

METHOD OF MAKING WATER-SOLUBLE  
CAPSULES FOR COSMETIC PURPOSES

Karl Wilhelm Schmidt, Nuremberg, Germany

No Drawing. Application March 8, 1938, Serial  
No. 194,641. In Germany November 26, 1937

1 Claim. (Cl. 167—85)

It is known to pack bathing-salts and cosmetic preparations in water-soluble capsules e. g. such made of urea, and to bring the filled capsule into the washing or bathing water, where the capsule dissolves, its contents getting thus into the water.

From this, the following facts have turned out: The cosmetic products contain perfume, ethereal oils and easily volatile substances. If such substances are filled into a capsule of the known kind, they diffuse comparatively quickly through the wall of the capsule, the surface of the capsule becomes insignificant, and the easily volatile substances vanish after a short time.

I have now found out, that this inconvenience can be partly done away with, if when pressing the capsules e. g. of urea, a pressure of at least 1000 kg/cm<sup>2</sup> is used, in order to fasten the walls of the capsule at a great extent. Capsules which are made in this way show a considerable density and satisfy the normal exigencies relating to their capability of being stored. For higher exigencies even this measure is not sufficient.

I have, however, succeeded in making an absolute dense capsule, by applying to its inner side a prepared layer. Such a layer must satisfy different exigencies: The layer must be a coherent film, it must vanish when the capsule dissolves in the bathing water, and it must not injure the smell nor react chemically with the contents of the capsule.

For this purpose of preparation, sodium stearate has proved to be well adapted, which, when brought upon the surface of the capsule in alcoholic solution and after having evaporated, gives a close layer. Instead of this compound, also sodium palmitate or sodium oleate may be used. Sodium resinate is usable, too. Furthermore, there may be taken hexene 1, 6-diol and urethane, which are favourable because of their low melting point and of their great water-solubility.

All these substances are water-soluble. There may, however, be taken such substances which are not water-soluble, but will melt in water of a slightly higher temperature, especially in the normal temperature of bathing water. I have found out, that a mixture of higher solid paraffines with a melting point of about 40° C., as e. g. nonadecane, eicosane, heneicosane and docosane, is suitable. The melting point of this mixture can be further lowered by melting together these substances with those links of the chemical series which have a lower melting point, the so-called paraffine oils. Furthermore are

apt for the given purpose: glycerides of palmitic acid, of stearic acid, and of oleic acid. The melting point of such a mixture is lowered according as the percentage of the glyceride of oleic acid is increased.

Substances of this kind can be placed upon the surface of the wall of the capsule in a melted state. By means of such an isolating layer, still other effects can be obtained. If hydro-aromatic compounds of the terpene series are used, the isolating layer itself can be made the aromatic substance or its bearer. So e. g. menthol has the property of melting at the temperature of the bathing water and of sticking to the skin. By this, a refreshing effect upon the body is obtained, similar to the one obtained by massage oils. Also terpine oil belongs to the substances of this class, its melting point being at 35° C.; it has the smell of elder, so that at the same time the bath is perfumed.

Instead of bringing the isolating means as a special layer upon the surface of the capsule to be pressed, this means can also be added to the pressing mass. For this, beside the said substances, also higher melting substances are suitable, because the process of pressing brings about a warming of the mass and may be executed under the supply of heat. E. g. a paraffine with a melting point of 40–60° C. can be added to the pressing mass in a quantity of 1–2%. By this small admixture, the solubility of the capsule is not diminished. In the same way, stearine may be applied. The admixtures are dissolved in a suitable solvent e. g. ether, and mixed to the pressing mass. After the ether is evaporated, the mass is ready to be worked up.

Capsules made of such a mass show no more the former drawbacks. Besides, there arises an advantage, as the pressure may be lower than would be necessary without the admixture. The scope of the employable substances is not limited by the above-named examples.

I claim:

A method of making water soluble capsules for cosmetic purposes, in which the content of the capsules is of easily volatile products, which consists in forming urea to the shape of a capsule, and subjecting the urea when so formed to capsule shape to a pressure of at least 1000 kg/cm<sup>2</sup>, to render the particles of urea forming the walls of the capsule impervious to the passage of volatile products, without destroying the inherent solubility of the capsule in water for exposing to the water the contents of the capsule.

KARL WILHELM SCHMIDT.